# EUROPEAN PATENT SPECIFICATION

(11) **EP 3 497 283 B1**
(45) Date of publication and mention of the grant of the patent: **03.08.2022**
(21) Application number: 17751579.8
(22) Date of filing: 04.08.2017
(51) Int. Cl.: D21H 27/00, D21H 19/36, D21H 19/82, B65D 65/38

(54) **OIL, GREASE, AND MOISTURE RESISTANT PAPERBOARD**
ÖL-, FETT- UND FEUCHTIGKEITSBESTÄNDIGE PAPPE
CARTON RÉSISTANT À L'HUILE, AUX GRAISSES ET À L'HUMIDITÉ

(30) Priority: 09.08.2016 US 201662372403 P; 07.09.2016 US 201615258181; 31.07.2017 US 201715664218
(43) Date of publication of application: 19.06.2019
(73) Proprietor: WestRock MWV, LLC, Atlanta, GA 30328 (US)
(72) Inventor: PARKER, Steven, Raleigh North Carolina 27606 (US); PANG, Jiebin, Glen Allen Virginia 23059 (US); MELTON, Natasha, Richmond Virginia 23221 (US)
(74) Representative: Coulson, Elizabeth Eve
(86) International application number: PCT/US2017/045414
(87) International publication number: WO 2018/031388

(56) References cited:
- WO-A1-96/05054
- US-A- 5 776 619
- US-A1- 2010 310 776
- US-B1- 6 548 120

## Description

### BACKGROUND OF THE INVENTION

### 1. Field of the Invention

This disclosure relates to paperboard substrates preferably having oil and grease resistance, yet with full recyclability and without having a tendency toward blocking, and furthermore being compostable.

### 2. Description of the Related Art

Sustainable packages using renewable, recyclable, and/or compostable materials are increasingly and strongly desired for food service and food packaging. Paper or paperboard itself is one of the most sustainable materials for packaging applications; however, paper or paperboard is often coated or laminated with barrier materials to fulfill the requirements of packaging. These additional barrier coatings or films often make the finished packages no longer repulpable or compostable. For example, widely used polyethylene coated paperboard is neither compostable nor recyclable under typical conditions. Polylactide coated paperboard can be compostable under industrial conditions, but it is not recyclable.

Oil and grease resistance is one of the top needs for paperboard packages in food and food service industries. Several technologies including specialty chemical (wax, fluorochemicals, starch, polyvinyl alcohol (PVOH), sodium alginate, etc.) treatment, polymer extrusion coating (polyethylene, etc.) have been employed to provide oil and grease resistance of paperboard packaging. However, the paper or paperboard treated with wax or coated with polyethylene, which is currently used in oil and grease resistant packaging, has difficulties in repulping and is not as easily recyclable as conventional paper or paperboard. Paper or paperboard treated with specialty chemicals such as fluorochemicals has potential health, safety and environmental concerns, and scientists have called for a stop to non-essential use of fluorochemicals in common consumer products including packaging materials.

There is a need for paperboard, especially oil and grease resistant paperboard, that is recyclable, compostable, low cost, and without environmental or safety concerns. Aqueous coating is one of the promising solutions to achieve these goals. However, blocking (the tendency of layers in a roll of paperboard to stick to one another) is a challenging technical hurdle in production and converting processes for aqueous barrier coated paperboard, and blocking is also a major technical hurdle for on-machine application of aqueous barrier coatings. Furthermore, most aqueous barrier coatings are not fully repulpable. Commonly-assigned United States application 15/017,735, published as U.S. Published Patent Application No. 2016-0230343 A1 addresses these problems. However, it is further desired to have a paperboard that is compostable. The ASTM D6868-11 Standard Specification for compostability of paper or paperboard requires any non-biodegradable organic constituent to be <1% of the dry weight of the finished product, and the total portion of organic constituents that are not biodegradable cannot exceed 5 % of the total weight. Most conventional or commercially available aqueous barrier coatings use high to pure synthetic polymer binder level, which makes it extremely challenging to meet this <1% non-biodegradable composition requirement for the ASTM compostability standard.

US 6548120 and US 2010/310776A disclose coated paper or paperboard products coated with a polymer which may optionally include starch. US 5776619 discloses multi-coated paperboard in which the preferred binder is n-alkyl-acrylate-acrylonitrile-styrene copolymer. These documents make no reference to compostability.

WO9605054A discloses a compostable paperboard comprising a primer coat and a top coat. The primer coat contains a polymer selected from acrylic polymer or copolymer, polyvinyl acetate, polyvinyl alcohol, poy-ethylene vinyl acetate, poly-ethylene vinyl chloride, styrene-butadiene copolymers, polyvinylidene chloride and starch. The top coat contains a polymer selected from acrylic polymer or copolymer, styrene-butadiene copolymers and polyvinylidiene chloride and imparts water and grease resistance. The coating preferably contains wax however. Furthermore most of the Examples omit pigment and there is no teaching regarding the pigment content.

### SUMMARY OF THE INVENTION

In one aspect the invention provides coated paperboard comprising:
a paperboard substrate having a first side and a second side;
a multilayer barrier coating having two or more layers in contact with the first side of the paperboard substrate, the multilayer coating comprising a base coating in contact with the paperboard substrate, the base coating having a coat weight from 9.76g/m2 to 16.26g/m2 (6 to 10 lbs per 3000 ft2) and comprising binder and pigment, and a top coating forming the outermost layer of the multilayer coating, the top coating having a coat weight from 4.88g/m2 to 16.26g/m2 (3 to 10 lbs per 3000 ft2) and comprising binder and pigment, the multilayer coating containing substantially no flurochemcial or wax;
wherein the pigment comprises at least one of a clay and calcium carbonate;
wherein the binder comprises one or more synthetic polymer binders and one or more additional natural biodegradable binders and wherein the additional biodegradable binder comprises between 1 to 10 parts per 100 parts pigment, by weight;
wherein the binder to pigment ratio in the multilayer coating is from about 25 to about 40 parts binder per 100 parts pigment, by weight;
wherein the coated paperboard has a caliper of at least 254µm (0.010"); and
wherein the coated paperboard is compostable according to the ASTM D6868-11 standard for compostability.

In another aspect the invention provides a method of treating paperboard, the method comprising:
providing a paperboard substrate having a first side and a second side;
applying to the first side a multilayer barrier coating having two or more layers, by applying a base coating in contact with the paperboard substrate, the base coating having a coat weight from 9.76g/m² to 16.26g/m² (6 to 10 lbs per 3000 ft²) and comprising binder and pigment, and applying a top coating forming the outermost layer of the multilayer coating, the top coating having a coat weight from 4.88g/m² to 16.26g/m² (3 to 10 lbs per 3000 ft²) and comprising binder and pigment, the multilayer coating containing substantially no fluorochemical or wax;
wherein the treated paperboard has a caliper of at least 254µm (0.010");
wherein the pigment comprises at least one of a clay and calcium carbonate;
wherein the binder comprises one or more synthetic polymer binders and one or more additional natural biodegradable binder and wherein the additional biodegradable binder comprises between 1 to 10 parts per 100 parts pigment, by weight;
wherein the binder to pigment ratio in the multilayer coating is from about 25 to about 40 parts binder per 100 parts pigment, by weight; and
wherein the treated paperboard is compostable according to the ASTM D6868-11 standard for compostability.

In a preferred embodiment the 'barrier' side of a paperboard is coated with at least one layer of aqueous coating containing a renewable natural material (modified starch) and a specialty synthetic binder, resulting in the coated oil and grease resistant paperboard (i.e., 254µm (10 pt caliper) and above) meeting the <1% non-biodegradable composition requirement for the compostability standard. The coating can be applied on a paper machine or by an off-line coater for example, and can optionally be applied in two coating steps (or two passes) for further enhanced barrier properties. Paperboard coated according to the invention preferably provides resistance to oil and grease and preferably does not have any tendency to block, and typically can be produced at a low cost.

Preferred embodiments of the invention are defined in the dependant claims.

### BRIEF DESCRIPTION OF THE DRAWINGS

FIG. 1 illustrates a method for producing a base stock on a paperboard machine;
FIG. 2 illustrates a method for treating the base stock from FIG. 1 by applying coatings to both sides on a paperboard machine;
FIG. 3 illustrates a method for treating the base stock from FIG. 1 by applying coatings to one side on a paperboard machine;
FIG. 4 illustrates a method for treating the base stock from FIG. 1 by applying coatings to one side on an off-machine coater;
FIG. 5 illustrates a device for measuring blocking of paperboard;
FIG. 6 is a graph of oil/grease resistance (3M kit level) vs. coat weight for several coatings; and
FIG. 7 is a graph of oil resistance (Cobb) vs. coat weight for several coatings.

### DETAILED DESCRIPTION OF THE INVENTION

FIG.1 and FIG 2 illustrate an exemplary on-paper machine method for coating a paperboard web with one or more layers of aqueous coating. A forming wire 110 in the form of an endless belt passes over a breast roll 115 that rotates proximate to a headbox 120. The headbox provides a fiber slurry in water with a fairly low consistency (for example, about 0.5% solids) that passes onto the moving forming wire 110. During a first distance 230 water drains from the slurry and through the forming wire 110, forming a web 300 of wet fibers. The slurry during distance 130 may yet have a wet appearance as there is free water on its surface. At some point as drainage continues the free water may disappear from the surface, and over distance 231, water may continue to drain although the surface appears free from water.

Eventually the web is carried by a transfer felt or press felt through one or more pressing devices such as press rolls 130 that help to further dewatering the web, usually with the application of pressure, vacuum, and sometimes heat. After pressing, the still relatively wet web 300 is dried, for example using dryer or drying sections 401, 402 to produce a dry web ("raw stock") 310 which may then be run through a size press 510 that applies a surface sizing to produce a sized "base stock" 320 which may then be run through additional dryer sections 403 and (on FIG. 2) smoothing steps such as calendar 520.

The base stock 320 may then be run through one or more coaters. For example, coater 530 may apply a first coat ("BC") to a first side ("C1") of the web, and the first coat may be dried in one or more dryer sections 404. Coater 540 may apply a second coat ("TC") to the first side of the web, and the second coat may be dried in one or more dryer sections 405.

If the web is to be coated on two sides, coater 550 may apply a first coat to the second side ("C2") of the web, and this coat may be dried in one or more dryer sections 406. Coater 560 may apply a second coat to the second side of the web, and this coat may be dried in one or more dryer sections 407. The order of coaters 540, 550 may be swapped, so that both sides C1 and C2 are first given a first coat, and then one side or both sides are given a second coat. In some instances, only one side will be coated as shown in FIG. 3, or only a first coat may be applied. In some instances, a third coat or more may be applied to one side.

Instead of applying coating by on-machine coaters as shown in FIGs. 2 and 3, coating may be applied by an off-machine coater as shown in Fig. 4. In such cases, the paperboard having been produced on the paper machine and wound onto reel 572 may then be transported (as a reel or as smaller rolls) to an off-machine coater 600, where the paperboard is unwound from reel 572, given a first coating by coater 610, dried in dryer(s) 601, given an optional second coating by coater 620, dried in dryer(s) 602, optionally given further treatment (such as gloss calendaring) and then wound onto reel 573. An off-machine coater could instead apply a single coat to one side of the paperboard, or could apply a single coat to each side, or could apply more than one coat to either or both sides. Alternately some coating may be done on the paper machine, with additional coating done on an off-machine coater.

Various types of coating devices may be used. The coaters illustrated in FIGs. 2 4 are devices where a coating is held in a pan, transferred by a roll to the lower surface of the web (which may be either the first side or the second side depending on the web path), and then the excess coating scraped off by a blade as the web wraps partially around a backing roll. However other coater types may be used instead, including but not limited to curtain coater, air knife coater, rod coater, film coater, short-dwell coater, spray coater, and metering film size press.

The particular materials used in the coatings may be selected according to the desired properties of the finished paperboard. For example, one side e.g. C1 may be given coating(s) that provide desired printability, while the other side e.g. C2 may be given barrier coating(s) that provide oil and grease resistance (OGR). The printability coating may be applied before the OGR coating, or, the OGR coating may be applied before the printability coating.

Following the coaters, there may be additional equipment for further processing such as additional smoothening, for example gloss calendaring. Finally, the web is tightly wound onto a reel 570.

The general process of papermaking and coating having been outlined at a high level in the preceding description and with Figures 1-4, we now turn to the coatings of the present invention. Typical aqueous barrier coatings often use specialty polymer(s), wax, and/or a higher polymer binder level (compared to conventional print coatings). These coatings can cause problems with repulpability of the coated paperboard because the coatings are usually difficult to breakdown to acceptable size or tend to form 'stickies' in paperboard making with the recycled fibers. Due to the high content of synthetic polymer binder in the coating, it is extremely challenging for each of the individual organic components in the coating to meet the <1% non-biodegradable composition requirement of the ASTM D6868-11 compostability standard.

Furthermore, many barrier coatings give paperboard a tendency to 'block' (the layers stick together) either in the reel 570, 571, 572, 573 or after it is rewound into rolls. Particularly in the reel 570, there may be residual heat from the dryers, which may dissipate quite slowly because of the large mass of the reel. Higher temperatures may increase the tendency toward blocking.

It is known that paperboard coated with conventional printability coatings usually does not block, and usually is fully repulpable. It would be advantageous if non-blocking and fully repulpable coatings also provided at least some degree of barrier properties. However, conventional printability coatings do not provide satisfactory barrier properties. Their formulations have relatively low levels of binder so as to absorb rather than repel fluid (printing ink, for example).

Binder amounts in conventional printability coatings can range from 15-25 parts per 100 parts of pigment by weight for base coatings, and 10-20 parts per 100 parts pigment by weight for top coatings. Printing grades would tend to be in the lower half of these ranges. Limiting the binder amount in the top coating may allow printing inks or adhesives to absorb readily into the printability coating. Simply increasing the binder to improve barrier properties eventually interferes with printability and causes additional problems, including blocking and repulpability problems.

Similar blocking and repulpability problems exist with many aqueous barrier coatings that use specialty polymer(s) and/or a higher polymer binder level (compared to printability coatings), with the deleterious effect that the coated paperboard is not completely recyclable and tends to block at elevated temperature or pressure.

In contrast, the inventive coatings disclosed in the present application meet the composition requirement for the ASTM compostability standard, and in preferred embodiments provide easy repulping, do not block at elevated temperature and pressure, and show good barrier properties, while using conventional pigments and synthetic and natural binders that are low-cost and readily available as coating materials for the paper or paperboard industry.

Conventional pigments may be used in the present invention and may include, but are not limited to, kaolin clay, calcium carbonate, etc. Pigments used in the examples herein are given the following 'shorthand' designations:
"Clay-1" kaolin clay, for example, a No. 1 ultrafine clay
"Clay-2" platy clay with high aspect ratio
"CaCO₃-1" coarse ground calcium carbonate (particle size 60% < 2micron)
"CaCO₃-2" fine ground calcium carbonate (particle size 90% < 2 micron)

Synthetic polymer binders may include, but are not limited to, styrene acrylate copolymer (SA), polyvinyl acetate (PVAc), and styrene-butadiene copolymer (SB), etc. Natural binders may include, but are not limited to, starch, alginate, protein, etc. Conventional styrene acrylate binder (SA, PHOPLEX^{®} C-340, available from Dow Chemical Company), acrylic polymer binder (Basonal^{®} X400AL, available from BASF Corporation), starch binder (Pen-cote^{®} D UHV, available from Ingredion Incorporated), or a blend of Pen-cote^{®} D with SA or Basonal^{®}, are used in examples described herein. Benefits of using Pen-cote^{®} D include its being directly dispersible into the formulation, increasing the coating formulation solids, and possibly being able to eliminate other thickeners. The choice of binder in the examples is not meant to be limiting in any way.

Coatings including control coatings were prepared according to the formulations shown in Table 1, which provides a list of major constituents in dry parts of the aqueous coating (C - Control, CF - Compostable Formulation) formulations used to achieve the oil and grease resistance, and to meet the composition requirement for the ASTM compostability standard, without blocking or repulpability problems. The test results are shown in Tables 3 and 4.

Substantially no fluorochemical was used in the coatings. By "substantially no fluorochemical" is meant that fluorochemicals were not deliberately utilized, and that any amount present would have been at most trace amounts. Although fluorochemicals can be excluded in lab experiments, trace amounts of such materials might be present in some paper machine systems due to making various grades of product, or might be introduced into a papermaking system through recycling processes. Likewise, substantially no wax was used in the coatings.

The total binder to pigment ratio (parts of binder, by weight, to 100 parts of pigment) of the formulations shown in Table 1 ranges from 30 to 35. This is more than the binder to pigment ratio for typical printability coatings (where rapid absorption of ink is desired) and less than the binder to pigment ratio of typical barrier coatings. Thus, it appears that an effective binder to pigment ratio may be from about 25 to about 40 parts binder per 100 parts pigment (by weight), or preferably from 30 to 35 parts binder per 100 parts pigment. Blending starch (such as Pen-cote@ D), a natural biodegradable material, into the formulation helps meet the <1% non-biodegradable composition requirement for the ASTM compostability standard while maintaining the barrier performance. The Pen-cote@ D starch was added at up to 5 parts in the final formulations.

Paperboard samples were made using solid bleached sulphate (SBS) substrate with a caliper of 457µm (18 pt., 0.018"). The samples were coated on one side (herein termed the "barrier side") using a pilot blade coater with a one-layer coating. The pilot results are expected to be representative of results that might be achieved on a production paper machine or a production off-machine coater.

The oil and grease resistance (OGR) of the samples was measured on the 'barrier side' by the 3M kit test (TAPPI Standard T559 cm-02). With this test, ratings are from 1 (the least resistance to oil and grease) to 12 (excellent resistance to oil and grease penetration). The results here gave 3M kit levels between 1 to 6 (see Table 3). The higher values were obtained with the higher coat weights for each specific formulation. Most interestingly, it is found that Basonal^{®} binder itself (C2 formulation) performs better on 3M kit level than SA binder (C1 formulation) at comparable coat weights (see Table 3); furthermore, blending Pen-cote^{®} D starch with Basonal^{®} (CF1-3) maintains the performance on 3M kit level as using Basonal^{®} itself at comparable or slightly higher coat weight, while meeting the <1% non-biodegradable composition requirement for the ASTM compostability standard. Especially, a 3M kit level of 4 5 (suitable for most food service packages) is achieved while meeting the compostability standard.

In addition to 3M kit test, oil absorptiveness (oil Cobb) was used to quantify and compare the OGR performance (oil and grease resistance), which measures the mass of oil absorbed in a specific time, e.g., 30 minutes, by 1 square meter of coated paperboard. For each condition tested, the sample was cut to provide two pieces each 162mm × 152mm (6 inch × 6 inch) square. Each square sample was weighed just before the test. Then a 102mm × 102mm, having an area of 0.0103 square metres (4 inch × 4 inch, having an area of 16 square inches) square of blotting paper saturated with peanut oil was put on the center of the test specimen (barrier side) and pressed gently to make sure the full area of oily blotting paper was contacting the coated surface. After 30-minutes as monitored by a stop watch, the oily blotting paper was gently removed using tweezers, and the excess amount of oil was wiped off from the coated surface using paper wipes (KimwipesTM). Then the test specimen was weighed again. The weight difference in grams before and after testing divided by the test area of 0.0103 square meters gave the oil Cobb value in grams/square meter.

As the oil Cobb results shown in Table 3, all the formulations (CF1-4) containing Basonal^{®} and Pen-cote^{®} D starch showed similar or improved (lower) oil Cobb value compared to both control formulations (C1 or C2), while all of them met the ASTM compostability standard. This confirmed the 3M kit results; and most interestingly, although CF4 at a coat weight 18.4 g/m² (11.3 lb/3msf) showed a 3M kit level of 3.8, it performed very well on actual oil holdout showing an oil Cobb of 4.9 gsm in 30 minutes (Table 3)

Moisture resistance of the coatings was evaluated by WVTR (water vapor transmission rate at 38°C and 90% relative humidity; TAPPI Standard T464 OM-12) and water Cobb (TAPPI Standard T441 om-04). All the formulations (CF1-4, Table 3) containing Basonal^{®} and Pen cote^{®} D starch showed similar water Cobb and WVTR values compared to both control formulations (C1 or C2), while all of them met the ASTM compostability standard.

The blocking behaviour of the samples was tested by evaluating the adhesion between the barrier coated side and the other uncoated side. A simplified illustration of the blocking test is shown in FIG. 5. The paperboard was cut into 51mm × 51mm (2" × 2") square samples. Several duplicates were tested for each condition, with each duplicate evaluating the blocking between a pair of samples 752, 754. (For example, if four duplicates were test, four pairs - eight pieces - would be used.) Each pair was positioned with the 'barrier-coated' side of one piece 752 contacting the uncoated side of the other piece 754. The pairs were placed into a stack 750 with a spacer 756 between adjacent pairs, the spacer being foil, release paper, or even copy paper. The entire sample stack was placed into the test device 700 illustrated in FIG. 5.

The test device 700 includes a frame 710. An adjustment knob 712 is attached to a screw 714 which is threaded through the frame top 716. The lower end of screw 714 is attached to a plate 718 which bears upon a heavy coil spring 720. The lower end of the spring 720 bears upon a plate 722 whose lower surface 724 has an area of one square inch. A scale 726 enables the user to read the applied force (which is equal to the pressure applied to the stack of samples through the one-square-inch lower surface 724).

The stack 750 of samples is placed between lower surface 724 and the frame bottom 728. The knob 712 is tightened until the scale 726 reads the desired force of 100 lbf (100 psi applied to the samples). The entire device 700 including samples is then placed in an oven at 50°C for 24 hours. The device 700 is then removed from the test environment and cooled to room temperature. The pressure is then released and the samples removed from the device.

The samples were evaluated for tackiness and blocking by separating each pair of paperboard sheets. The results were reported as shown in Table 2, with a 0 rating indicating no tendency to blocking.

Blocking damage is visible as fiber tear, which if present usually occurs with fibers pulling up from the non-barrier surface of samples 754. If the non-barrier surface was coated with a print coating, then blocking might also be evinced by damage to the print coating.

For example, in as symbolically depicted in FIG. 5, samples 752(0)/754(0) might be representative of a "0" blocking (no blocking). The circular shape in the samples indicates an approximate area that was under pressure, for instance about one square inch of the overall sample. Samples 752(3)/754(3) might be representative of a "3" blocking rating, with up to 25% fiber tear in the area that was under pressure, particularly in the uncoated surface of sample 754(3). Samples 752(4)/754(4) might be representative of a "4" blocking rating with more than 25% fiber tear, particularly in the uncoated surface of sample 754(4). The depictions in FIG. 5 are only meant to approximately suggest the percent damage to such test samples, rather than showing a realistic appearance of the samples.

Repulpability was tested using an AMC Maelstom repulper. 110 grams of coated paperboard, cut into 25mm × 25mm (1"×1") squares, was added to the repulper containing 2895 grams of water (pH of 6.5±0.5, 50°C), soaked for 15 minutes, and then repulped for 30 minutes. 300 mL of the repulped slurry was then screened through a Vibrating Flat Screen (0.15mm (0.006") slot size). Rejects (caught by the screen) and fiber accepts were collected, dried and weighed. The percentage of accepts was calculated based on the weights of accepts and rejects, with 100% being complete repulpability.

As an example of poor repulpability, SBS paperboard coated with low density polyethylene (LDPE) at a coat weight of 11.4 - 17.9 g/m² (7-11 lbs per 3000ft²) was tested and gave fiber accepts in a range of 91 to 97%. (A fiber accepts percentage close to 100% is desired). Paperboard coated with polyethylene not easily repulpable and recyclable.

Various coating formulations shown in Table 1 were applied as single layers onto a paperboard substrate, using a range of coat weights, and the results are shown in Table 3 including repulpability and compostability. All of the samples were fully repulpable. As for compostability, as seen in the first two columns of Table 3, paperboard C1 with coating using a pure styrene acrylate (SA) binder did not meet the definition of compostable at coat weights of 14.7 - 16.3 g/m² (9-10 pounds). Furthermore, these C1 samples blocked slightly, whereas the other samples did not. The next two columns show that paperboard C2 with coating using a Basonal^{®} X 400 AL binder (made by BASF Corporation) met the definition of compostability at a coat weight of 13.0 g/m² (8 pounds), but not at a coat weight of 14.6 g/m² (9 pounds.) The last four columns (paperboard CF1, CF2, CF3, CF4) are for coatings blending the Basonal^{®} binder with Pen-cote^{®} D, a modified starch made by Ingredion Incorporated. These paperboards all meet the compostability definition.

Also included in Table 3 are measurements of Gloss, Brightness, Whiteness, and L-a-b Color. Gloss was measured on a Technidyne Model T 480A Glossmeter according to TAPPI standard T480. (GE) Brightness was measured on a Technidyne Brightimeter Micro S-5 according to TAPPI standard T452. (CIE) Whiteness was measured the Technidyne Brightimeter Micro S-5 according to TAPPI standard T562. L-a-b color was measured on the Technidyne Brightimeter Micro S-5 according to TAPPI standard T524. Using Basonal^{®} binder or a blend of Basonal^{®} binder with Pen-cote^{®} D starch showed similar or slightly higher gloss of the coating than using SA binder, but with slightly lower brightness and whiteness and slightly higher b-color value. Barrier properties are the focus of the inventive coatings, however, if there is a need to adjust the color or shade, food contact compliant dyes can be used in the formulations.

Another experiment was done by applying the CF3 formulation in two passes on a blade coater, with the first layer coat weight of 9.3 g/m² (5.7 lb/3msf) and the second layer coat weight of4.9 g/m² (3.0 lb/3msf), resulting a total coat weight of only 14.2 g/m² (8.7 lb/3msf), which met the composition requirement for compostability standard and showed a 3M kit value of 6.0. As shown from Table 4, a kit level of 5.2 was obtained when a single layer of CF3 was applied with a higher coat weight of 15.8 g/m² (9.7 lb/3msf). These results demonstrated that enhanced barrier properties can be obtained with two passes of the barrier formulations.

The Basonal^{®} X 400 AL binder made by BASF Corporation contains about 30% natural polymer component. A natural polymer component refers to one grown and found in nature, which for example, can be any protein or polysaccharide or their derivatives. The idea of using the Basonal^{®} X 400 AL binder along with some additional natural polymer (such as starch) in the present invention was that the natural component in the Basonal^{®} binder would promote the compatibility of the additional starch with the Basonal^{®} binder. Compatibility of the different ingredients is important for a barrier coating. To prove the concept, additional tests were run as shown in Table 4 to compare SA binder (PHOPLEX^{®} C-340 from Dow Chemical Company used in the examples) and Basonal^{®} X 400 AL (from BASF Corporation), both including Pen cote^{®} D starch in the formulations at a same blend ratio. All of the samples were fully repulpable and non-blocking. As for compostability, as seen in the first three columns of Table 4, paperboard C3 with coating using a styrene acrylate (SA) / Pen-cote^{®} D binder did not meet the definition of compostability at coat weights of 13.0 - 19.5 g/m² (8-12 pounds). The next three columns show that paperboard CF3 with coating using a Basonal^{®} binder and Pen-cote^{®} D met the definition of compostability at a coat weight of 13.0 g/m² and 15.8 g/m² (8.0 and 9.7 pounds), but not at a high coat weight of 17.6 g/m² (10.8 pounds). Most interestingly, the CF3 (Basonal^{®} + Pen-cote^{®} D) coatings had better OGR and moisture vapor barrier performance, in other words, higher 3M kit and lower Oil Cobb values, lower WVTR values, and approximately equal water Cobb values, compared to the C3 (SA + Pen-cote^{®} D) coatings. Tables 3 and 4 thus show that the combined use of Pen-cote^{®} D specialized starch with Basonal^{®} binder provides improved barrier performance, especially, achieving a 3M kit level of 5+, while meeting the compostability standard, being fully repulpable, and not having blocking problems.

As another way to visualize the test results, the data were plotted as shown in FIGs. 6 and 7. Some of the data on the graphs comes from Tables 3 and 4. Other data are also included. FIG. 6 shows 3M kit level vs. coat weight. The kit value generally increases (improves) as coat weight increases. None of the control samples (using SA binder) were compostable in the coat weight range of 9.8-19.5 g/m² (6-12 lbs / 3msf). The samples (CF2 and CF3) using 35 parts of (combined) Basonal^{®} X400AL binder plus Pen-cote^{®} D starch were compostable except at the highest coat weights (16.6 g/m² (10.2 lbs) for CF2 and 17.6 g/m² (10.8 lbs /3msf) for CF3) and gave kit values equal to or better (higher) than the control SA sample at comparable coat weight. Samples using 30 parts of (combined) Basonal^{®} and Pen-Cote^{®} D were all compostable (at least up to at least 18.7 g/m² (11.5 lbs / 3msf)), while their kit values tended to be lower than the control and the other samples.

FIG. 7 shows oil Cobb vs. coat weight for the selected samples as in FIG. 6. The oil Cobb generally decreases (improves) as coat weight increases. The compostability (or lack thereof) has already been described. The test samples using (combined) Basonal^{®} and Pen-cote^{®} D gave oil Cobb tests equal or better (lower) than the test samples using styrene-acrylate binder. Most interestingly, for the samples with a total 30 parts of binder (25 parts Basonal^{®} and 5 parts of Pen-cote^{®} D), although the 3M kit values were lower than the other formulations with 35 total parts of binder (as FIG. 6), the oil Cobb values were still similar or better than the control sample C1 with 35 parts of pure SA binder. This again proves the synergistic effect of Basonal^{®} with Pen-cote^{®} D starch.

Some food service or food packaging applications require high quality printing on the external side of the package in addition to a barrier for the food contact side. To demonstrate that a finished paperboard with a barrier coating on one side and a print coating on the other side can meet the composition requirements for the ASTM compostability standard, another experiment was conducted to test print coat formulations that used conventional binders, styrene acrylate (PHOPLEX^{®} C-340 used, available from Dow Chemical Company) and polyvinyl acetate (POLYCO^{™} 2160 used, available from Dow Chemical Company), with each polymer binder in the coatings meeting the <1% non-biodegradable composition requirement for 305µm (caliper 12 pt) and above, according to the compostability standard ASTM D6868-11. Although the print coat formulations for these tests were adjusted slightly by reducing the content of SA binder, the coatings still showed high quality of printability comparable to that of the commercial print grade.

The printable formulations that were tested are summarized in Table 5 for three base coatings and two top coatings described using a basis of 100 parts pigment. Table 6 shows coat weights used in several pilot coater tests for the printable formulations on 458µm (18 pt) paperboard. Paperboards with the printable test coatings shown in Table 6 all would be compostable according to the ASTM standard, provided the paperboard caliper is 305µm (12 pts) or higher. This would be true with - or without - the compostable barrier coatings (described above) on the opposite side of the paperboard.

Table 6 also shows the roughness, optical properties, and printability results for the test coatings. Optical properties including Gloss, Brightness, Whiteness, and L-a-b color were measured according to TAPPI standards described above. Parker Print-Surf (PPS) roughness was measured according to TAPPI standard T555. The coated samples were printed on a Harper Phantom QD^{™} Flexo Proofing System from Harper Corporation using a 2.5 bcm anilox roll with a blue flexo ink. The ink density was measured on an X-Rite 500 series equipment. All test coatings, which would be compostable showed higher gloss, slightly higher brightness, and comparable whiteness over the commercial control. No dyes were used in the test coatings, which in addition to variables in the formulations could contribute to the slight difference of L-a-b color values. All the test coatings showed relatively higher PPS values over the commercial control; however, they were still fairly good, and all of the test coatings after printing showed ink density slightly higher (1.64-1.72 vs. 1.62) than the commercial control, indicating the good printability of the printable test coatings. For the printability tests, a barrier coating was not applied to the opposite side of the paperboard. However, calculations show that the printable paperboard would meet the compostability standard ASTM D6868-11, whether or not the earlier-described compostable barrier coatings were used on the side opposite from the printable coating. Although two layers of printable coatings (base coat and top coat) were used in the examples, one layer of printable coating is also possible to provide fair printability and also meet the compostability standard.

In summary, the results show that compostable paperboard with full repulpability and moderate grease resistance is achieved by replacing standard binders (such as styrene acrylate) with a binder such as Basonal^{®} X400AL in combination with small amounts of Pen-cote^{®} D specialized starch. In combination with conventional clay coatings that use standard binders (such as styrene acrylate and polyvinyl acetate) on the non-barrier (print) side, which also meet the <1% composition threshold for each non-biodegradable organic constituent, the entire finished paperboard product meets the composition requirements of compostability standard, at least for paperboards of caliper 305µm (12 pt and higher). The compostability standard involves calculations of how much of each non-biodegradable organic constituent is used in the product. It is hypothesized that by adjusting the coating, or the paperboard basis weight, compostability according to the ASTM standard might be achieved with somewhat lower calipers, such as 254µm (10 pt. (0.010")). It is also hypothesized that by selecting multiple different binders, with or without biodegradable polymer binders, compostability according to the ASTM standard can be achieved for paperboard with printable coatings on both sides, where the paperboard has a caliper of 254µm (10 pt) and higher.

The tests described above used a blade coater to apply coating. As previously discussed, various types of coating devices may be used.

Once given the above disclosure, many other features, modifications or improvements will become apparent to the skilled artisan. Such features, modifications or improvements are, therefore, considered to be a part of this invention, the scope of which is to be determined by the following claims.

While preferred embodiments of the invention have been described and illustrated, it should be apparent that many modifications to the embodiments and implementations of the invention can be made without departing from the scope of the invention. It is to be understood therefore that the invention is not limited to the particular embodiments disclosed (or apparent from the disclosure) herein, but only limited by the claims appended hereto.

**TABLE 1.**

| **Coating Formulations** | | | | | | | |
|---|---|---|---|---|---|---|---|
| **Designation** | **C1** | **C2** | **C3** | **CF1** | **CF2** | **CF3** | **CF4** |
| Clay-1 | 25 | 25 | 25 | 25 | 25 | 25 | 25 |
| Clay-2 | 50 | 50 | 50 | 50 | 50 | 50 | 50 |
| CaCO₃-1 | 25 | 25 | 25 | 25 | 25 | 25 | 25 |
| PHOPLEX^{®} C-340(SA) | 35 | | 30 | | | | |
| Basonal^{®} X400AL | | 35 | | 33 | 32 | 30 | 25 |
| Pen-cote^{®} D UHV (starch) | | | 5 | 2 | 3 | 5 | 5 |
| binder/pigment ratio | 35/100 | 35/100 | 35/100 | 35/100 | 35/100 | 35/100 | 30/100 |

**TABLE 2.**

| **Blocking Ratings** | |
|---|---|
| 0 | = samples fall apart without any force applied |
| 1 | = samples have a light tackiness but separate without fiber tear |
| 2 | = samples have a high tackiness but separate without fiber tear |
| 3 | = samples are sticky and up to 25% fiber tear or coat damage (area basis) |
| 4 | = samples have more than 25% fiber tear or coat damage (area basis) |

**TABLE 3.**

| **Effect of Various Binders on Coating Properties including Compostability** | | | | | | | | | |
|---|---|---|---|---|---|---|---|---|---|
| **Designation →** | **C1 SA** | | **C2 Basonal^{®}** | | | **Basonal CF1 Basonal + Pen-cote D** | **CF2 Basonal + Pen-cote D** | **CF3 Basonal + Pen-cote D** | **CF4 Basonal + Pen-cote D** |
| **Coat wt g/m²** (lb/3msf) | 14.5 (8.9) | 15.6 (9.6) | 13.2 (8.1) | 14.6 (9.0) | | 13.7 (8.4) | 14.5 (8.9) | 15.8 (9.7) | 18.4 (11.3) |
| **Compostable** ^{∗} | No | No | Yes | No | | Yes | Yes | Yes | Yes |
| **Repulp** % accepts | - | 100 | - | 100 | | 100 | 100 | 100 | - |
| **3M kit** | 2.8 | 5.4 | 3.6 | 4.6 | | 4.0 | 5.0 | 5.2 | 3.8 |
| **Oil Cobb** grams / (m² 30min) | 23.7 | 10.2 | 17.5 | 9.4 | | 11.3 | 12.3 | 6.1 | 4.9 |
| **H2O Cobb** grams / (m² 2min) | 30.2 | 30.3 | 32.9 | 32.4 | | 31.2 | 30.3 | 29.8 | 30.9 |
| **WVTR** grams / (m² day) | 891 | 764 | 829 | 758 | | 773 | 839 | 790 | 909 |
| **Blocking** | 1 | 1 | 0 | 0 | | 0 | 0 | 0 | 0 |
| **Gloss** | 13.5 | 14.0 | - | 13.8 | | - | 14.5 | 16.0 | 16.6 |
| **Brightness** | 79.5 | 79.4 | - | 76.2 | | - | 76.1 | 75.5 | 76.3 |
| **Whiteness** | 66.8 | 66.3 | - | 58.2 | | - | 57.9 | 56.3 | 57.8 |
| **L-a-b** Color | 91.0 | 91.9 | - | 91.2 | | - | 90.1 | 90.0 | 90.3 |
| | 0.4 | 0.4 | | 0.2 | | | 0.2 | 0.2 | 0.2 |
| | 3.4 | 3.5 | | 4.8 | | | 4.9 | 5.1 | 5.0 |
| ^{∗} Compostable: defined as less than 1% by weight of non-biodegradable constituent for paperboard calipers of 12 points or higher | | | | | | | | | |

**TABLE 4. Compostability with SA & Basonal^{®} (Pen-cote^{®} D added to both)**

| **Designation →** | **C3 SA + Pen-cote^{®} D** | | | **CF3 Basonal^{®} + Pen-cote^{®} D** | | | | | |
|---|---|---|---|---|---|---|---|---|---|
| **Coat wt g/m²** (lb/3msf) | 13.5 (8.3) | 16.4 (10.1) | 18.9 (11.6) | 13.0 (8.0) | 15.8 (9.7) | 17.6 (10.8) | | | |
| **Compostable** | No | No | No | Yes | Yes | No | | | |
| **Repulp** % accepts | - | 100 | 100 | - | 100 | 100 | | | |
| **3M kit** | 1.2 | 1.8 | 2.8 | 2.6 | 5.2 | 6.2 | | | |
| **Oil Cobb** grams / (m² 30min) | 46.5 | 14.9 | 6.1 | 45.5 | 6.1 | 2.3 | | | |
| **H2O Cobb** grams / (m² 2min) | - | 26.6 | 28.4 | 31.1 | 29.8 | 31.3 | | | |
| **WVTR** grams / (m² day) | - | 915 | 930 | 959 | 790 | 680 | | | |
| **Blocking** | 0 | 0 | 0 | 0 | 0 | 0 | | | |

**TABLE 5. Formulations for Printable Coatings**

| **Designation** | **BC1** | **BC2** | **BC3** | **TC1** | **TC2** |
|---|---|---|---|---|---|
| **Clay-1** | | | | 51 | 30 |
| **Clay-2** | 50 | | | | |
| **CaCO₃-1** | 50 | 100 | 100 | | |
| **CaCO₃-2** | | | | 49 | 70 |
| **PHOPLEX^{®} C-340 (SA)** | 19 | 17 | 17 | 4 | 5 |
| **POLYCO^{™} 2160 (PVAc)** | 6 | 4 | | 12 | 11 |
| **Pen-cote^{®} D UHV (starch)** | | | 4 | | |

**TABLE 6. Printability Tests on Printable Coatings**

| (18 pt paperboard; no barrier coating on opposite side) | | | | | | | | | |
|---|---|---|---|---|---|---|---|---|---|
| **Designation → BC Coat wt** g/m² (lb/3msf) | **Commercial Control** 15.3 (9.4) | **BC1/ TC1** 14.3 (8.8) | **BC2/ TC1** 12.2 (7.5) | **BC2/ TC1** 11.7 (7.2) | **BC2/ TC2** 12.2 (7.5) | **BC2/ TC2** 12.2 (7.5) | **BC3/ TC1** 10.1 (6.2) | **BC3/ TC1** 10.4 (6.4) | **BC3/ TC2** 10.4 (6.4) |
| **TC Coat wt** g/m² (lb/3msf) | 7.6 (4.7) | 8.8 (5.4) | 11.7 (7.2) | 5.4 (3.3) | 11.6 (7.1) | 13.3 (8.2) | 11.6 (7.1) | 14.6 (9.0) | 12.4 (7.6) |
| **Compostable** ∗ **Parker PrintSurf** | No 1.47 | Yes 1.50 | Yes 1.80 | Yes 2.51 | Yes 1.94 | Yes 2.27 | Yes 1.82 | Yes 1.92 | Yes 1.87 |
| **Gloss** | 46.6 | 56.4 | 57.1 | 48.9 | 52.2 | 50.3 | 57.5 | 59.2 | 51.1 |
| **Brightness** | 83.5 | 84.6 | 84.9 | 83.5 | 85.5 | 85.0 | 85.0 | 84.4 | 85.5 |
| **Whiteness** | 77.4 | 75.9 | 77.0 | 73.9 | 78.6 | 76.9 | 77.3 | 75.4 | 78.8 |
| **L-a-b** Color | 92.0 -0.4 1.6 | 93.2 0.4 2.4 | 93.2 0.5 2.2 | 92.7 0.1 2.6 | 93.3 0.5 1.8 | 93.3 0.2 2.2 | 93.2 0.4 2.1 | 93.2 0.1 2.5 | 93.3 0.5 1.8 |
| **Ink Density** | 1.62 | 1.64 | 1.71 | 1.73 | 1.72 | 1.68 | 1.71 | 1.70 | 1.71 |

| | | | | | | | | | |
|---|---|---|---|---|---|---|---|---|---|
| (^{∗}Compostable: defined as less than 1% by weight of non-biodegradable constituent for paperboard calipers of 12 points or higher) | | | | | | | | | |

## Claims

1. A coated paperboard comprising:
a paperboard substrate having a first side and a second side;
a multilayer coating having two or more layers in contact with the first side of the paperboard substrate, the multilayer coating comprising a base coating in contact with the paperboard substrate, the base coating having a coat weight from 9.76g/m² to 16.26g/m² (6 to 10 lbs per 3000 ft²) and comprising binder and pigment, and a top coating forming the outermost layer of the multilayer coating, the top coating having a coat weight from 4.88g/m² to 16.26g/m² (3 to 10 lbs per 3000 ft²) and comprising binder and pigment, the multilayer coating containing substantially no fluorochemical or wax;
wherein the pigment comprises at least one of a clay and calcium carbonate;
wherein the binder comprises one or more synthetic polymer binders and one or more additional natural biodegradable binders and wherein the additional biodegradable binder comprises between 1 to 10 parts per 100 parts pigment, by weight;
wherein the binder to pigment ratio in the multilayer coating is from about 25 to about 40 parts binder per 100 parts pigment, by weight;
wherein the coated paperboard has a caliper of at least 254µm (0.010"); and
wherein the coated paperboard is compostable according to the ASTM D6868-11 standard for compostability.

2. The coated paperboard of claim 1, wherein the top coating has a coat weight from 6.51g/m² to 11.39g/m² (4 to 7 lbs per 3000 ft²).

3. The coated paperboard of claim 1 or 2, wherein the total coat weight of the multilayer coating is from 8.14g/m² to 19.53g/m² (5 to 12 lbs per 3000 ft²).

4. The coated paperboard of any of claims 1 to 3, wherein the multilayer coating is further applied in contact with the second side of the paperboard substrate.

5. The coated paperboard of any of claims 1 to 4, wherein the multilayer coating has two layers, and wherein the top coating is formed in contact with the base coating.

6. The coated paperboard of any of claims 1 to 5, wherein the multilayer coating is a printable coating.

7. The coated paperboard of any preceding claim, wherein the multilayer coating is an oil and grease-resistant (OGR) coating.

8. The coated paperboard of any preceding claim, wherein the additional biodegradable binders include at least one of polysaccharide, protein, and derivatives thereof.

9. The coated paperboard of any preceding claim, wherein the additional biodegradable binder comprises starch.

10. The coated paperboard of any preceding claim, wherein the coated paperboard is repulpable to the extent that after repulping the percentage accepts is at least 99%.

11. The coated paperboard of any preceding claim, having no tendency toward blocking after being held for 24 hours at 50°C at a pressure of 689kPa (100 psi).

12. A method of treating paperboard, the method comprising:
providing a paperboard substrate having a first side and a second side;
applying to the first side a multilayer coating having two or more layers, by applying a base coating in contact with the paperboard substrate, the base coating having a coat weight from 9.76g/m² to 16.26g/m² (6 to 10 lbs per 3000 ft²) and comprising binder and pigment, and applying a top coating forming the outermost layer of the multilayer coating, the top coating having a coat weight from 4.88g/m² to 16.26g/m² (3 to 10 lbs per 3000 ft²) and comprising binder and pigment, the multilayer coating containing substantially no fluorochemical or wax;
wherein the treated paperboard has a caliper of at least 254µm (0.010");
wherein the pigment comprises at least one of a clay and calcium carbonate;
wherein the binder comprises one or more synthetic polymer binders and one or more additional natural biodegradable binders and wherein the additional biodegradable binder comprises between 1 to 10 parts per 100 parts pigment, by weight;
wherein the binder to pigment ratio in the multilayer coating is from about 25 to about 40 parts binder per 100 parts pigment, by weight; and
wherein the treated paperboard is compostable according to the ASTM D6868-11 standard for compostability.

13. The method of claim 12, wherein the multilayer coating is as defined in any of claims 2 to 6 and 8.

14. The method of claim 12 or claim 13, wherein the treated paperboard is repulpable to the extent that after repulping the percentage of accepts is at least 99%.

## Patentansprüche

1. Beschichtete Pappe, umfassend:
ein Pappsubstrat mit einer ersten Seite und einer zweiten Seite;
eine Mehrlagenbeschichtung mit zwei oder mehr Lagen, die in Kontakt mit der ersten Seite des Pappsubstrats stehen, wobei die Mehrlagenbeschichtung eine Basisschicht umfasst, die in Kontakt mit dem Pappsubstrat steht, wobei die Basisschicht ein Schichtgewicht von 9,76 g/m² bis 16,26 g/m² (6 bis 10 lbs pro 3000 ft²) hat und ein Bindemittel sowie ein Pigment umfasst, und die Mehrlagenbeschichtung ferner eine Deckschicht umfasst, die die äußerste Schicht der Mehrlagenbeschichtung bildet, wobei die Deckschicht ein Schichtgewicht von 4,88 g/m² bis 16,26 g/m² (3 bis 10 lbs pro 3000 ft²) hat und ein Bindemittel sowie ein Pigment umfasst, und wobei die Mehrlagenbeschichtung im Wesentlichen keine Fluorchemikalien oder Wachse enthält;
wobei das Pigment wenigstens entweder Ton oder ein Calciumcarbonat umfasst;
wobei das Bindemittel ein oder mehrere synthetische Polymerbindemittel umfasst und ein oder mehrere zusätzliche natürliche biologisch abbaubare Bindemittel, und wobei das zusätzliche biologisch abbaubare Bindemittel zwischen 1 und 10 Gewichtsanteilen pro 100 Pigment-Gewichtsanteilen umfasst;
wobei das Verhältnis von Bindemittel zu Pigment in der Mehrlagenbeschichtung von etwa 25 bis etwa 40 Bindemittel-Gewichtsanteilen pro 100 Pigment-Gewichtsanteilen liegt;
wobei die beschichtete Pappe eine Stärke von wenigstens 254 µm (0,010") aufweist; und
wobei die beschichtete Pappe gemäß der Norm ASTM D6868-11 für Kompostierbarkeit kompostierbar ist.

2. Beschichtete Pappe nach Anspruch 1, wobei die Deckschicht ein Schichtgewicht von 6,51 g/m² bis 11,39 g/m² (4 bis 7 lbs pro 3000 ft²) hat.

3. Beschichtete Pappe nach Anspruch 1 oder 2, wobei das Gesamtschichtgewicht der Mehrlagenbeschichtung im Bereich von 8,14 g/m² bis 19,53 g/m² (5 bis 12 lbs pro 3000 ft²) liegt.

4. Beschichtete Pappe nach einem der Ansprüche 1 bis 3, wobei die Mehrlagenbeschichtung ferner in Kontakt mit der zweiten Seite des Pappsubstrats aufgebracht wird.

5. Beschichtete Pappe nach einem der Ansprüche 1 bis 4, wobei die Mehrlagenbeschichtung zwei Lagen aufweist und wobei die Deckschicht in Kontakt mit der Basisschicht ausgebildet ist.

6. Beschichtete Pappe nach einem der Ansprüche 1 bis 5, wobei die Mehrlagenbeschichtung eine bedruckbare Beschichtung ist.

7. Beschichtete Pappe nach einem der vorhergehenden Ansprüche, wobei die Mehrlagenbeschichtung eine öl- und fettbeständige (OGR) Beschichtung ist.

8. Beschichtete Pappe nach einem der vorhergehenden Ansprüche, wobei die zusätzlichen biologisch abbaubaren Bindemittel wenigstens eines von Polysacchariden, Proteinen und Derivaten davon umfassen.

9. Beschichtete Pappe nach einem der vorhergehenden Ansprüche, wobei das zusätzliche biologisch abbaubare Bindemittel Stärke umfasst.

10. Beschichtete Pappe nach einem der vorhergehenden Ansprüche, wobei die beschichtete Pappe in dem Maße wiederaufbereitbar ist, dass der Prozentsatz der Akzeptanz nach dem Wiederaufbereiten wenigstens 99 % beträgt.

11. Beschichtete Pappe nach einem der vorhergehenden Ansprüche, die nicht zum Verblocken neigt, nachdem sie 24 Stunden lang einer Temperatur von 50°C und einem Druck von 689 kPa (100 psi) ausgesetzt wurde.

12. Verfahren zum Behandeln von Pappe, wobei das Verfahren umfasst:
Bereitstellen eines Pappsubstrats mit einer ersten Seite und einer zweiten Seite;
Aufbringen einer Mehrlagenbeschichtung mit zwei oder mehr Lagen auf die erste Seite durch Aufbringen einer Basisschicht in Kontakt mit dem Pappsubstrat, wobei die Basisschicht ein Schichtgewicht von 9,76 g/m² bis 16,26 g/m² (6 bis 10 lbs pro 3000 ft²) hat und ein Bindemittel sowie ein Pigment umfasst, und Aufbringen einer Deckschicht, die die äußerste Schicht der Mehrlagenbeschichtung bildet, wobei die Deckschicht ein Schichtgewicht von 4,88 g/m² bis 16,26 g/m² (3 bis 10 lbs pro 3000 ft²) hat und ein Bindemittel sowie ein Pigment umfasst, wobei die Mehrlagenbeschichtung im Wesentlichen keine Fluorchemikalien oder Wachse enthält;
wobei die behandelte Pappe eine Stärke von wenigstens 254 µm (0,010") aufweist;
wobei das Pigment wenigstens entweder Ton oder Calciumcarbonat umfasst;
wobei das Bindemittel ein oder mehrere synthetische Polymerbindemittel und ein oder mehrere zusätzliche natürlich biologisch abbaubare Bindemittel umfasst und wobei das zusätzliche biologisch abbaubare Bindemittel zwischen 1 und 10 Gewichtsanteilen pro 100 Pigment-Gewichtsanteilen umfasst;
wobei das Verhältnis von Bindemittel zu Pigment in der Mehrlagenbeschichtung im Bereich von etwa 25 bis etwa 40 Bindemittel-Gewichtsanteilen pro 100 Pigment-Gewichtsanteilen liegt; und
wobei die behandelte Pappe gemäß der Norm ASTM D6868-11 für Kompostierbarkeit kompostierbar ist.

13. Verfahren nach Anspruch 12, wobei die Mehrlagenbeschichtung nach einem der Ansprüche 2 bis 6 und 8 definiert ist.

14. Verfahren nach Anspruch 12 oder Anspruch 13, wobei die behandelte Pappe in dem Maße wiederaufbereitbar ist, dass der Prozentsatz der Akzeptanz nach dem Wiederaufbereiten wenigstens 99 % beträgt.

## Revendications

1. Carton couché comprenant :
un support en carton ayant une première face et une seconde face ;
un couchage multicouche comportant deux ou plus de deux couches en contact avec la première face du support en carton, le couchage multicouche comprenant un couchage de fond en contact avec le support en carton, le couchage de fond ayant un poids de couche de 9,76 g/m² à 16,26 g/m² (6 à 10 livres pour 3 000 pieds²) et comprenant liant et pigment, et un couchage de finition formant la couche la plus externe du couchage multicouche, le couchage de finition ayant un poids de couche de 4,88 g/m² à 16,26 g/m² (3 à 10 livres pour 3 000 pieds²) et comprenant liant et pigment, le couchage multicouche ne contenant pratiquement pas de composé chimique fluoré ni de cire ;
dans lequel le pigment comprend au moins un(e) parmi une argile et le carbonate de calcium ;
dans lequel le liant comprend un ou plusieurs liant(s) polymère(s) synthétique(s) et un ou plusieurs liant(s) biodégradable(s) naturel(s) supplémentaire(s) et le liant biodégradable supplémentaire représentant entre 1 et 10 parties pour 100 parties de pigment, en poids ;
dans lequel le rapport liant à pigment dans le couchage multicouche vaut d'environ 25 à environ 40 parties de liant pour 100 parties de pigment, en poids ;
dans lequel le carton couché a une épaisseur d'au moins 254 µm (0,010 pouce) ; et
dans lequel le carton couché est compostable conformément à la norme de compostabilité ASTM D6868-11.

2. Carton couché selon la revendication 1, dans lequel le couchage de finition a un poids de couche de 6,51 g/m² à 11,39 g/m² (4 à 7 livres pour 3 000 pieds²).

3. Carton couché selon la revendication 1 ou 2, dans lequel le poids de couche total du couchage multicouche vaut de 8,14 g/m² à 19,53 g/m² (5 à 12 livres pour 3 000 pieds²).

4. Carton couché selon l'une quelconque des revendications 1 à 3, dans lequel le couchage multicouche est en outre appliqué en contact avec la seconde face du support en carton.

5. Carton couché selon l'une quelconque des revendications 1 à 4, dans lequel le couchage multicouche comporte deux couches, et dans lequel le couchage de finition est formé en contact avec le couchage de fond.

6. Carton couché selon l'une quelconque des revendications 1 à 5, dans lequel le couchage multicouche est un couchage apte à recevoir une impression.

7. Carton couché selon l'une quelconque des revendications précédentes, dans lequel le couchage multicouche est un couchage résistant aux huiles et aux graisses (RHG).

8. Carton couché selon l'une quelconque des revendications précédentes, dans lequel les liants biodégradables supplémentaires incluent au moins un(e) parmi un polysaccharide, une protéine, et leurs dérivés.

9. Carton couché selon l'une quelconque des revendications précédentes, dans lequel le liant biodégradable supplémentaire comprend l'amidon.

10. Carton couché selon l'une quelconque des revendications précédentes, dans lequel le carton couché est apte à être remis en pâte jusqu'au degré où après remise en pâte le pourcentage de pâte acceptée est d'au moins 99 %.

11. Carton couché selon l'une quelconque des revendications précédentes, n'ayant pas de tendance à l'adhérence en surface après avoir été maintenu pendant 24 heures à 50 °C sous une pression de 689 kPa (100 psi).

12. Procédé de traitement de carton, le procédé comprenant les étapes consistant à :
fournir un support en carton ayant une première face et une seconde face ;
appliquer sur la première face un couchage multicouche comportant deux ou plus de deux couches, en appliquant un couchage de fond en contact avec le support en carton, le couchage de fond ayant un poids de couche de 9,76 g/m² à 16,26 g/m² (6 à 10 livres pour 3 000 pieds²) et comprenant liant et pigment, et appliquer un couchage de finition formant la couche la plus externe du couchage multicouche, le couchage de finition ayant un poids de couche de 4,88 g/m² à 16,26 g/m² (3 à 10 livres pour 3 000 pieds²) et comprenant liant et pigment, le couchage multicouche ne contenant pratiquement pas de composé chimique fluoré ni de cire ;
dans lequel le carton couché a une épaisseur d'au moins 254 µm (0,010 pouce) ;
dans lequel le pigment comprend au moins un(e) parmi une argile et le carbonate de calcium ;
dans lequel le liant comprend un ou plusieurs liant(s) polymère(s) synthétique(s) et un ou plusieurs liant(s) biodégradable(s) naturel(s) supplémentaire(s) et le liant biodégradable supplémentaire représentant entre 1 et 10 parties pour 100 parties de pigment, en poids ;
dans lequel le rapport liant à pigment dans le couchage multicouche vaut d'environ 25 à environ 40 parties de liant pour 100 parties de pigment, en poids ; et
dans lequel le carton couché est compostable conformément à la norme de compostabilité ASTM D6868-11.

13. Procédé selon la revendication 12, dans lequel le couchage multicouche est tel que défini dans l'une quelconque des revendications 2 à 6 et 8.

14. Procédé selon la revendication 12 ou la revendication 13, dans lequel le carton couché est apte à être remis en pâte jusqu'au degré où après remise en pâte le pourcentage de pâte acceptée est d'au moins 99 %.
